

## UNITED STATES PATENT OFFICE

2,429,574

## CARBOCYANINES FROM ALICYCLICDIOXY AZOLES

Alfred W. Anish, Johnson, and Lee C. Hensley, Binghamton, N. Y., assignors to General Aniline & Film Corporation, New York, N. Y., a corporation of Delaware

No Drawing. Original application August 16, 1944, Serial No. 549,789. Divided and this application August 16, 1944, Serial No. 549,788

8 Claims. (Cl. 260—240)

1

The present invention relates to new compounds of the thio and seleno-carbocyanine type and to a method of preparing the same.

In certain processes of subtractive multi-color photography a multi-layer photographic material is used in which the lowest light-sensitive layer is sensitive only for red above 6000 A. U. (in the region of the threshold of sensitivity). This red-sensitive layer must always be insensitive to blue-green light since the presence of blue-green sensitivity gives rise to falsification of color. In all color-photography processes in which the color of the component pictures is produced by color development, there may be present in the photographic layer in addition to the sensitizer a color former which, when the exposed silver halide emulsion is developed, combines with the oxidation product of the developer to form a sparingly soluble dye distributed in the layer proportionately to the quantity of silver image. In this case, a sensitizer must be selected, the effect of which is not enfeebled by the presence of the dye component. Sensitizers are already known which have a high intensity in the red region of the spectrum but, these for the most part are enfeebled by the presence of a dye component.

It is known that many carbocyanines of which the 5, 6-position of the benzene nucleus is occupied, sensitize photographic silver halide emulsions to high red sensitivity. Most of these carbocyanines, however, are not suitable for sensitizing silver halide emulsions containing color coupling components. This is thought to be due to a physical displacement which the sensitizing dye undergoes when color coupling components are added. That is, the sensitizer is adsorbed to the surface of the silver halide grain, and then, with addition of color component, is displaced therefrom.

An object of the present invention is to provide a class of sensitizers which are free from the disadvantages noted above.

A further object is to provide a new class of thio and seleno-carbocyanines containing a hydrogenated ring system as a part of the cyanine dye molecule.

A further object involves a method of preparing such thio and seleno-carbocyanines.

A still further object is to provide thio and seleno-carbocyanines which are added to photo-

2

graphic emulsions, or coated thereon as an over-coating, whereby the sensitivity of the photographic emulsion is increased.

Other objects and advantages of this invention will become apparent by reference to the following specification in which its preferred details and embodiments are described.

This invention is based on the discovery that thio and seleno-carbocyanines containing a 10 cyclic hydrocarbon substituted dioxy ring structure as part of the cyanine dye molecule not only sensitizes a photographic silver halide emulsion to high red sensitivity, but are also compatible with color coupling components for the cyan dye image. In the latter combination the sensitizing action of the dyes is not impaired or diminished. In addition to these desirable characteristics, it has been further found that when used in conjunction with color coupling components for the 15 blue-green image, the spectral curves of these dyes show a desirable gap in the green region of the spectrum—that is, the dye sensitivity is more selective to the red spectral region. The sensitizing capacity of these dyes is not only maintained in the presence of color formers for the blue-green image, especially those color formers containing long chain hydroxyalkyl groups, but is increased, and in part rendered more selective. This entirely new property is most surprising and 20 wholly unexpected. An additional advantage of these dyes is their ability to remain fixed in the one layer in which they are originally deposited.

The sensitizing dyes suitable for the purpose of the present invention have the general 25 formula:



wherein R represents the methylene groups 40 necessary to complete at least a 5-membered alicyclic ring system such as cyclopentylidene, cyclohexylidene, cycloheptylidene, and the like, R<sub>1</sub> and R<sub>2</sub> are alkyl groups, e. g., methyl, ethyl, propyl, butyl, amyl, etc., Y represents sulfur or 45 selenium, X represents an acid radical, e. g., Cl, 50

Br, I, SO<sub>4</sub>, ClO<sub>4</sub>, SO<sub>4</sub>CH<sub>3</sub>, SO<sub>4</sub>C<sub>2</sub>H<sub>5</sub>, SO<sub>3</sub>C<sub>2</sub>H<sub>4</sub>CH<sub>3</sub> and the like, and Z represents a grouping of atoms necessary to complete a heterocyclic ring usual in the cyanine dye art, such as indolenine, thiazole, benzthiazole, benzselenazole and the like; these rings may be substituted by alkyl as above, aryl, e. g., phenyl, naphthyl or anthranyl, alicyclic ring system of the same value as R, alkoxy, e. g., methoxy, ethoxy, propoxy, butoxy, etc., alkylidioxy, or cycloalkyl dioxy nuclei.

These sensitizing dyes are obtained by condensing quaternary ammonium salts of thiazoles and selenazoles containing an alicyclic dioxy ring such as cyclopentylidenedioxy, cyclohexylidenedioxy, or cycloheptylidenedioxy ring as a part of the nucleus with ethyl-orthoformate or with 2-( $\beta$ -acetanilido vinyl)-5, 6-methylenedioxybenzthiazole ethiodide, 2-( $\beta$ -acetanilido vinyl)-5, 6-cyclohexylidenedioxybenzthiazole ethiodide, or the corresponding seleno derivatives thereof.

The alicyclicdioxybenzenes used in preparing the alicyclicdioxybenzthiazoles and alicyclicdioxybenzselenazoles which are condensed with any one of the above listed intermediates or coupling agents, are readily prepared by reacting catechol with a cyclic ketone as described in Recueil Travaux Chimiques des Pays Bas, vol. 54, p. 997 (1935).

The following examples describe in detail the methods for accomplishing the above objects, but it is to be understood that they are inserted merely for the purpose of illustration, and are not to be construed as limiting the scope of the invention.

*Example I*

3,3'-diethyl-5,6-5',6'-dicyclohexylidenedioxy-benzthiocarbocyanine iodide



Cyclohexylidenedioxybenzene was prepared according to the above publication by dissolving

had a boiling point of 125° C. at 12 mm. M. P. 44° C.

The cyclohexylidenedioxybenzene was converted to 1,2-dinitro-4,5-cyclohexylidenedioxybenzene by treating the former with a mixture of glacial acetic and fuming nitric acids. The resulting product was then converted to the disulfide by treating it in 200 cc. of boiling ethyl alcohol with a fused mixture of equivalent quantities of sodium sulfide nonahydrate and sulfur in small portions until a violet color persisted for a few minutes. The solid was filtered from the cool mixture, washed alternately with water and alcohol, and dried.

Nine gms. of the disulfide was added to a mixture consisting of 28 cc. of acetic anhydride, 22 cc. of glacial acetic acid and 3 cc. of acetyl chloride, and heated on a steam bath. Eleven gms. of zinc dust was then added in small portions with stirring to the heated mixture. The free base was precipitated from the acid reaction mixture by pouring into 6 volumes of cold water. The 2-methyl-5,6-cyclohexylidenedioxybenzthiazole was filtered, dried and had a melting point of 140-142° C. The ethyl-p-toluenesulfonate salt was made in the usual manner and had a melting point of 169° C.

0.69 gm. of the quaternary salt thus prepared was treated with 0.5 cc. of ethyl-orthoformate in 30 5 gms. of pyridine in the presence of a trace of triethylamine at 130-140° C. for 3 hours. Upon cooling, 20 cc. of water was added. After standing overnight, the solid that separated was dissolved in 15 cc. of hot n-propyl alcohol and the 35 solution treated with 3 cc. of 20% potassium iodide solution, filtered and allowed to cool. The dye precipitated on standing. It was filtered off, and after washing with water, the dye was recrystallized from ethyl alcohol as the iodide. The 40 crystals melted above 250° C.

Incorporated in a gelatino silver halide emulsion containing about 4-5% of silver halide, the dye sensitized to about 6800 Å., with a maximum sensitivity at 6400 Å.

Twenty milligrams of the sensitizing dye prepared as above was dissolved in 50 cc. of methyl alcohol, and added to one kilogram of silver halide gelatin emulsion containing about 10% gelatin, 4-5% of silver halide and 12.0 gms. of N-octadecyl-1-hydroxy-2-naphthoylamine. The coated 50 emulsion had a maximum red sensitivity at about 6650 Å., and developed to a blue-green image with p-phenylenediamine developer. The sensitizing dye did not diffuse in multi-layer coatings.

*Example II*

3,3'-diethyl-5,6-cyclohexylidenedioxy-5',6'-methylenedioxy-benzthiocarbocyanine iodide



55 gms. of catechol in 100 gms. of hot anhydrous cyclohexanone and treated with an excess of phosphoric anhydride (125 gms.). After the addition was completed, the stirring was continued for a short time, and the upper layer decanted. The decanted material was mixed with 150 cc. of a dilute solution of sodium carbonate and steam-distilled. The distillate was extracted with ether and the dried solvent evaporated. The residue of the cyclohexylidenedioxybenzene was distilled at reduced pressure and the resulting distillate

65 250 milligrams of 2-( $\beta$ -acetanilido vinyl)-5,6-methylenedioxybenzthiazole ethiodide prepared by heating at 135° C. a mixture of equal weight portions of 2-methyl-5,6-methylenedioxybenzthiazole ethiodide and diphenyl formamidine in acetic anhydride for forty minutes were mixed 70 with an equal amount of 2-methyl-5,6-cyclohexylidenedioxybenzthiazole ethyl-p-toluenesulfonate prepared according to Example I, in 5 cc. of pyridine and 3 drops of triethylamine. The 75 mixture was heated to reflux for 1 hour, cooled,

and an equal volume of water added. The dye crystals which separated out on standing were filtered off and recrystallized from ethyl alcohol.

Incorporated in a gelatino silver halide emulsion containing about 4-5% of silver halide, the dye sensitized to about 6850 Å., with a maximum sensitivity at 6420 Å.

Twenty-five milligrams of the sensitizing dye

phenylenediamine developer. The dye did not diffuse in multi-layer coatings.

When 8.0 gms. of 1-hydroxy 2,4-dichloronaphthalene were substituted for 12.0 gms. of N-octadecyl-1-hydroxy-2-naphthoylamine, the coated emulsion showed a high red sensitivity, and developed to a blue-green image with a p-phenylenediamine developer.

#### Example IV

##### 3,3'-Diethyl-5,6-5',6'-dicyclopentylidenedioxy-benzthiocarboxylic acid iodide



above prepared was dissolved in 50 cc. of methyl alcohol, and added to a kilo of silver halide gelatin emulsion containing about 10% gelatin, 4-5% of silver halide, and 12 gms. of 3,5-di(phenylamino) phenol. The coated emulsion showed a high red sensitivity, and developed to a blue-green image with a p-phenylenediamine developer.

- 20 5.3 gms. of 2-methyl-5,6-cyclopentylidenedioxybenzthiazole ethyl-p-toluenesulfonate, prepared in a manner similar to the corresponding 2-methyl-5,6-cyclohexylidenedioxybenzthiazole in Example I, and five gms. of ethyl-orthoformate were refluxed in 20.0 cc. of pyridine for 2½ hours. An equal volume of water was added and the dye which separated was filtered off, washed

#### Example III

##### 3,3'-diethyl-5,6-cyclohexylidenedioxy-5',6'-methylenedioxy-benzthiobenzselenocarboxylic acid iodide



0.8 gm. of 2-( $\beta$ -acetanilido vinyl)-5,6-cyclohexylidenedioxybenzthiazole ethiodide and 0.6 gm. of 2-methyl-5,6-methylenedioxybenzthiobenzselenocarboxylic acid ethyl-p-toluenesulfonate were mixed with 25 cc. of pyridine and 0.5 cc. of triethylamine added. The mixture was refluxed for 1½ hours. The dye solution was diluted with water and allowed to stand overnight. The dye crystals which separated were filtered off and washed with water, and recrystallized from ethyl alcohol.

Incorporated in a gelatino silver halide emulsion containing about 4-5% of silver halide, the

- 40 with water, and crystallized from methyl alcohol. Incorporated in a gelatino silver halide emulsion containing 4-5% of silver halide, the dye sensitized to about 6800 Å., with a maximum sensitivity at 6400 Å.
- 45 Twenty-five milligrams of the sensitizing dye prepared as above was added to a kilo of silver halide gelatin emulsion containing about 10% gelatin, 4-5% of silver halide, and 10 gms. of 8-hydroxyquinoline as the color former. The 50 coated emulsion showed a high red sensitivity, and developed to a blue-green image with a p-phenylenediamine developer.

#### Example V

##### 3,3'-Diethyl-5,6-cyclohexylidenedioxy-6',7'-benzobenzthiocarboxylic acid iodide



dye sensitized to about 6850 Å., with a maximum sensitivity at 6450 Å.

Twenty-five milligrams of the sensitizing dye prepared as above was added to a kilo of silver halide gelatin emulsion containing about 10% gelatin, 4-5% of silver halide and 12.0 gms. of N-octadecyl-1-hydroxy-2-naphthoylamine. The coated emulsion showed a high red sensitivity, and developed to a blue-green image with a p-

- 5.4 gms. of 2-( $\beta$ -acetanilido vinyl)-5,6-cyclohexylidenedioxybenzthiazole ethiodide was mixed with 4.0 gms. of 2-methyl-6,7-benzobenzothiophene ethyl-p-toluenesulfonate, 20.0 cc. pyridine and 4.0 cc. triethylamine. The mixture was heated to reflux for one hour, cooled, and an equal volume of water added. The dye crystals which separated out on standing were filtered off and recrystallized from methyl alcohol.

Incorporated in a gelatino silver halide emulsion containing 4-5% of silver halide, the dye sensitized to about 6800 Å., with a maximum sensitivity at 6400 Å.

Twenty-five milligrams of the sensitizing dye prepared as above was added to a kilo of silver halide gelatin emulsion, containing about 10% gelatin, 4-5% of silver halide, and 10 gms. of  $\alpha$ -hydroxydiphenyl as the color former. The coated emulsion showed a high red sensitivity, and developed to a blue-green image with a p-phenylenediamine developer.

*Example VI*

3,3'-diethyl-5,6-cyclohexylidenedioxy-5',6'-dimethoxybenzothiocarbocyanine iodide



5.4 gms. of 2-( $\beta$ -acetanilido vinyl)-5,6-cyclohexylidenedioxybenzothiazole ethiodide was mixed with 4.2 gms. of 2-methyl-5,6-dimethoxybenzothiazole ethyl-p-toluenesulfonate, 20 cc. of pyridine and 4 cc. of triethylamine. The mixture was heated to reflux for one hour, cooled, and an equal amount of water added. The dye crystals which separated out on standing were filtered off and recrystallized from methyl alcohol.

Incorporated in a gelatino silver halide emulsion containing about 4-5% of silver halide, the dye sensitized to about 6800 Å., with a maximum sensitivity at 6400 Å.

Twenty-five milligrams of the sensitizing dye prepared as above, was added to a kilo of silver halide gelatin emulsion containing about 10% gelatin, 4-5% of silver halide, and 12 gms. of  $\alpha$ -hydroxy naphthoic acid as the color former. The coated emulsion showed a high red sensitivity, and developed to a blue-green image with a p-phenylenediamine developer.

In the preparation of silver halide emulsions containing the sensitizing dyes of the present invention, the dyes may be dissolved in methyl or ethyl alcohol and a volume solution containing from 5 to 50 milligrams of the dye added to a liter of emulsion. While in general practice it may not be necessary to add the dye in larger amounts, generally, for satisfactory results, amounts usually ranging from 5 to 25 milligrams are sufficient to obtain the maximum sensitizing effect. However, we do not wish to limit our invention to the quantities just indicated; the most suitable amount will in each case be found by a few comparative experiments. The dyes may be added to the emulsion in form of solutions. In actual practice, the dyes are applied to the emulsion during any stage of its production; however, they are preferably added to the finished emulsion before being cast.

tion, since it will be apparent to those skilled in the art, that the dyes may be incorporated into photographic emulsions by methods other than those described herein.

This application is a division of our co-pending application Serial No. 549,789 filed on even date.

While there have been pointed out above certain preferred embodiments of the invention, the same is not limited to the foregoing examples, illustrations, or to the specific details given therein, but is capable of variations and modifications

25 as to the reactants, proportions and conditions employed. Accordingly, it is intended that the invention be defined only by the accompanying claims, in which it is intended to include all features of patentable novelty residing therein.

30 We claim:

1. Compounds of the general formula:



wherein R represents the methylene groups necessary to complete at least a 5-membered alicyclic ring system, R<sub>1</sub> and R<sub>2</sub> represent an alkyl group, X represents an acid radical, Y represents a member taken from the class consisting of sulfur and selenium, and Z represents the atoms necessary to complete a nitrogenous heterocyclic ring system of the type usual in cyanine dyes.

2. The chemical compound 3,3'-diethyl-5,6,5',6'-dicyclohexylidenedioxybenzothiocarbocyanine iodide having the following formula:



3. The chemical compound 3,3'-diethyl-5,6,5',6'-dicyclopentylidenedioxybenzothiocarbocyanine iodide having the following formula:



4. The chemical compound 3,3'-diethyl-5,6-cyclohexylidenedioxy-5',6'-dimethoxybenzothiocarbo-

The above examples are illustrative only, and should not be construed as limiting the invention.

9

carbocyanine iodide having the following formula:



5. A process of preparing thio and seleno-carbocyanine dyes containing a cyclic hydrocarbon substituted dioxy ring structure as part of the cyanine dye molecule which comprises reacting a member selected from the class of alicyclicdioxypyrazoles and alicyclicdioxypyrazoles with a member selected from the class consisting of ethyl-orthoformate and a cyclammonium quaternary salt, having an active group in the  $\beta$ -position and selected from the class consisting of alkyl mercapto and aryl acyl amino groups under the influence of heat in the presence of a basic condensing agent.

6. A process of preparing a thio-carbocyanine containing a cyclohexylienedioxy ring structure as part of the cyanine dye molecules, which comprises reacting under the influence of heat, one mol of 2-methyl-5,6-cyclohexylienedioxybenzthiazole ethyl-p-toluenesulfonate with one mol of 2-( $\beta$ -acetanilido vinyl)-5,6-methylenedioxybenzthiazole ethiodide in the presence of a basic condensing agent.

7. A process of preparing a thio-seleno carbocyanine containing a cyclohexylidenedioxy

10

ring structure as part of the cyanine dye molecule, which comprises reacting under the influ-

- 15 ence of heat, one mol of 2-methyl-5,6-methylene-dioxybenzselenaazole ethyl-p-toluenesulfonate with one mol of 2-( $\beta$ -acetanilido vinyl)-5,6-cyclohexylidenedioxybenzthiazole ethiodide in the presence of a basic condensing agent.

20 8. A process of preparing a thio-carbocyanine containing a cyclopentylidenedioxy ring structure as part of the cyanine dye molecule, which comprises reacting under the influence of heat, one mol of 2-methyl-5,6-cyclopentylidenedioxybenzthiazole ethyl-p-toluenesulfonate with one mol of ethylorthoformate in the presence of a basic condensing agent.

ALFRED W. ANISH.  
LEE C. HENSLEY.

#### REFERENCES CITED

- 30 The following references are of record in the file of this patent:

UNITED STATES PATENTS

35 Number Name Date  
2,334,711 Kendall ----- Nov. 23, 1943  
2,126,078 Zeh ----- Aug. 9, 1938